

# UNITED STATES PATENT OFFICE.

ERNST WIRTH, OF DORTMUND, GERMANY, ASSIGNOR, BY MESNE ASSIGNMENTS, TO  
THE CHEMICAL FOUNDATION, INC., A CORPORATION OF DELAWARE.

## PRODUCING RESINOUS BASES FROM TAR.

1,339,310.

Specification of Letters Patent.

Patented May 4, 1920.

No Drawing. Application filed May 20, 1916, Serial No. 99,254. Renewed August 6, 1919. Serial No. 315,785.

To all whom it may concern:

Be it known that I, ERNST WIRTH, manufacturer, a subject of the German Emperor, and residing at Dortmund, in the German Empire, have invented certain new and useful Improvements in Producing Resinous Bases from Tar, of which the following is a specification.

The present invention relates to a process for producing from mineral coal tar and other tars, from tar products and tar oils hitherto unknown resinous bases with a high boiling point. Heretofore only acridine had been found in mineral coal tar as a base boiling above 300° cent. and the existence of other bases with high boiling temperatures was unknown. I have now found that there exist further bases, about 3%, with high boiling temperatures both in mineral coal tar and in tar oils with a high boiling point, which bases can, however, not be obtained by a simple treatment with acids, as their salts form insoluble compounds with phenol, its higher homologues and naphthols and other tar components, which compounds make up the greater portion of the acid-tar produced by the acid treatment of the tar. If, however, the phenols are previously removed from the tar or the tar oils, for example by treatment with alkalis, the bases may, to the greater part, be removed directly by aid of acids, while a small part forms with unknown tar components a resinous material, from which the salts of the bases may be removed by boiling in water. From the solution of the salts the bases may be precipitated in form of a viscous mass by aid of a suitable lye. The bases commence to boil at about 320° cent. whereas the last components pass over in *vacuo* only at more than 400° cent. By fractional distillation in *vacuo* they may thereupon be separated. The components of a low boiling point may be separated in the same manner from the tar oils boiling above 300° cent., the components with a higher boiling point from the pitch remaining from the distillation of coal tar. The lower fractions are yellow oils, the medium ones viscous, and the fractions with the highest boiling temperatures solid reddish brown substances. Neither the bases nor their

plain salts may be obtained in a crystallized form. They show a similarity to the bases of the formula  $C_nH_{2n-11}N$  found by Robinson and Goodwin in the acid tar from shale oil (*Transact. Royal Soc. Edinburgh*, 1878 p. 561 and 1879 p. 265), but differ therefrom by a considerably lower contents of hydrogen and have the formula  $C_{2n+1}H_{n+3}N$ . 55 60

The lowest boiling fraction has the composition  $C_{13}H_9N$  but contains none of the two known naphthoquinolins; it consists besides acridine probably of naphthoquinolins which were unknown heretofore. 65 These bases may be used for manufacturing pharmaceutical products and in the dye-stuff industries; the components of the highest boiling point, probably anthraisoquinolins and similar bases, will directly dye 70 wool and silk from a yellow to a brownish red color.

In order to obtain the said bases from the coal tar the following method is preferably employed: 100 kilos of tar is freed of 75 the most valuable components as benzene, its homologues, phenol and pyridin, and, if it is too viscous for filtration, is diluted with about 50 kilos of a coal tar oil which has been previously freed of phenols and bases. 80 The tar is then freed from the free carbon contained therein by settling or filtration and treated in a mixer at a suitable temperature with caustic soda solution of a specific gravity of 1.15 in such a quantity that 85 all phenols are dissolved, as for instance, 10 liters. After settling, the soda lye containing the phenols is drawn off and the remaining tar is well stirred with 10 liters of dilute sulfuric acid of a specific gravity of 90 1.12. When settled, the aqueous solution containing the sulfates of the new bases is drawn off at the bottom. After cooling, the coal tar purified by this treatment can be separated from the formed resinous material 95 solidified during the cooling process. The resinous material is boiled with water in order to extract the sulfates of the new bases mixed with it. The sulfate solutions of the new bases are neutralized with caustic soda in order to render the new bases insoluble in water. The bases can be isolated by fractional distillation, preferably 100 in *vacuo*. The first runnings contain quin-

olin and its homologues, boiling at 236 to about 290° cent. At 320° C. the new bases begin to come over together with the acridine which may be separated by repeated 5 fractional distillations.

In the same manner the bases can be extracted from the heavy coal tar oils boiling above 300° cent. and also from coal tar pitch, which must be diluted with a larger 10 quantity of light coal tar oil.

The tar freed from these bases consists of a viscid dark brown oil which even when highly heated will not be decomposed or 15 form coke, and which is therefore excellently suited for heating and also as a lubricant.

I claim:

1. Process of recovering resinous bases having a high boiling point from tar, consisting 20 in distilling off the phenols, diluting it with coal tar, previously freed of phenols, removing the carbon by filtration, treating the product with a caustic soda solution, removing the soda lye, stirring the product with 25 diluted sulfuric acid, removing the sulfates, cooling the mass, and separating the pure tar from the resinous material contained in

the mixture and finally isolating the bases from said resinous material by fractional distillation, substantially as described. 30

2. The process of recovering resinous bases having a high boiling point from tar, which comprises distilling off the phenols, diluting it with coal tar, previously freed from phenols, removing the carbon by filtration, treating the product with a caustic solution, removing the lye, stirring the product with diluted sulfuric acid, removing the sulfates, cooling the mass, separating the pure tar from the resinous material 35 contained in the mixture, extracting said resinous material with water to remove the soluble bases in the form of sulfates, treating the sulfate solutions with caustic alkali, and finally isolating the bases from the insoluble material thus produced by fractional 40 distillation, substantially as described.

In testimony whereof I have affixed my signature in presence of two witnesses.

ERNST WIRTH. [L. s.]

Witnesses:

HELEN NUFER,  
ALBERT NUFER.